

## UNITED STATES PATENT OFFICE

2,669,764

MANUFACTURE OF MICACEOUS  
INSULATING MATERIALS

James S. Kilpatrick, Cirencester, England, assignor to The Mycalex Company Limited, Cirencester, England, a British company

No Drawing. Application May 1, 1950,  
Serial No. 159,379

5 Claims. (Cl. 25—156)

1

This invention relates to micaceous insulating materials of the kind which are formed by mixing low fusing point vitreous material with powdered mica and heating the mixture so that the mica is bonded to the vitreous material at a temperature below the point of total dehydration. An example of such material is that known under the registered trade-mark "Mycalex" whose manufacture is described inter alia in the specification of United States Patent No. 2,303,244.

The object of the present invention is to provide a new form of material having the general character described in the preceding paragraph but which possesses, in addition to the dielectric and other advantageous properties of such material, the capability of being formed into a variety of articles by injection moulding in a more expeditious and economical manner than has been possible hitherto with materials of the general class above described.

According to the invention a method of manufacturing a micaceous insulating material is provided which consists in mixing a white glass frit with barium carbonate and phlogopite mica, in forming the mixture into billets or blocks, in subjecting the billets or blocks to a rise in temperature in a furnace and in moulding and cooling the heat treated material.

In carrying the invention into effect and in the preferred manner, a mixture is prepared consisting of a white glass frit, barium carbonate and phlogopite mica. The frit consisting of cryolite, barium carbonate, potassium carbonate, soda ash and boric acid may be and preferably is formed as described in the aforesaid U. S. specification No. 2,303,244. Alternatively, the frit may be prepared from the ingredients in the proportions as follows:

|                  | Per cent |
|------------------|----------|
| Barium carbonate | 46.75    |
| Boric acid       | 20.00    |
| Aluminium oxide  | 0.25     |
| Phlogopite mica  | 33.00    |

All the ingredients of the mixture are initially ground to a particle size capable of passing a mesh of 100 x 100 per square inch. In preparing the mixture the preferred proportions of the ingredients, that is of the frit, the barium carbonate and the phlogopite mica, consist in one third of each by weight but, although the proportions may be varied, it has been found essential for the best results in the finished articles that the proportions of the frit and the phlogopite mica should be equal. For satisfactory re-

2

sults, the proportions by weight of the frit and the phlogopite mica should not be greater than 45% of each nor less than 30% of each. After thoroughly mixing the said ingredients they are formed into billets, a small proportion of water being added to assist in forming a coherent body under the moulding pressure.

After formation, as described, the billets are allowed to dry for a period up to five days in length. To assist in rendering the material coherent and capable of readily forming into billets a small proportion of methyl cellulose or dextrine may be added to the water and being volatile, this added matter disappears when the material is heat treated as hereinafter described.

After the billets have been dried they are furnace treated to a temperature of the order of 850 degrees C. the time of treatment varying with the weight of the billet treated. It has been found in practice that on the average the time of heat treatment required is about 7 minutes per ounce weight of the billet treated. From the furnace the billets are transferred directly to an injection moulding apparatus which may conveniently be of one of the forms described in the specification of our British Patent No. 601,772. It is essential, however, for satisfactory results to be obtained that the temperature of the mould shall be maintained at from 300 to 350 degrees centigrade and that the moulded articles produced shall be cooled slowly.

The process above described may be modified by including lead oxide in the proportion of 10% by weight with the barium carbonate, as although this addition adds somewhat to the cost of production, it has the advantage of enabling the mould temperature to be reduced to one of the order of 300 degrees centigrade.

The invention possesses the advantage that in comparison with previously known processes for producing an injection moulding material of the "Mycalex" class, the production costs are reduced as are also the power factor and the specific gravity of the products. The lowering of the specific gravity approximately to 2 is an important advantage in that the weight of the material, as compared with previous products of a similar character, is approximately halved for a given volume, thereby rendering the products adapted for aircraft and for other uses where weight is an important factor.

I claim:

1. The method of manufacturing a micaceous insulating material characterized by its injection moulding properties comprising in mixing a white

glass frit with barium carbonate and phlogopite mica, in forming the mixture into billets or blocks, in subjecting the billets or blocks to a rise in temperature in a furnace and in moulding and cooling the heat treated material said frit, barium carbonate and mica being each employed in the proportion of substantially one-third by weight.

2. The method of manufacturing an article a micaceous insulating material characterized by its injection moulding properties comprising in heating a mixture of cryolite, barium carbonate, potassium carbonate, soda ash and boric acid to form a white glass frit, in mixing said frit with barium carbonate and phlogopite mica, in grinding the mixture to fine particle size, in forming the ground ingredients into billets under pressure, in heating said billets and in injection moulding the heat treated material said frit, barium carbonate and mica being each employed in the proportion of substantially one-third by weight.

3. The method according to claim 1 wherein approximately ten per cent lead oxide is included with the barium carbonate.

4. The method as defined in claim 2 wherein

approximately ten per cent lead oxide is included with the barium carbonate.

5. In the method of manufacturing billets of a micaceous insulating material suitable for injection moulding, the steps of preparing a mixture of finely ground white glass frit, barium carbonate and phlogopite mica, the frit and the phlogopite mica being present in substantially equal proportions, forming the said mixture into billets under pressure, allowing the billets to dry and subjecting the dried billets to heat treatment in a furnace up to a temperature in the neighborhood of 850° C., transferring the billets from the furnace to an injection mold maintained at a temperature of from 300 to 500° C., molding the billets in the injection mold, and allowing the injection molded products to cool slowly.

JAMES S. KILPATRICK.

References Cited in the file of this patent

UNITED STATES PATENTS

| Number    | Name    | Date          |
|-----------|---------|---------------|
| 2,032,239 | Wedlock | Feb. 25, 1936 |
| 2,303,244 | Wedlock | Nov. 24, 1942 |